

I. LADOFF.  
ARC LIGHT ELECTRODE.  
APPLICATION FILED JUNE 1, 1907.

1,025,407.

Patented May 7, 1912.



Witnesses:  
C. A. Jangs  
Philip Beck

Inventor:  
Isidor Ladoff.  
By Walter Diamond  
attorney.

# UNITED STATES PATENT OFFICE.

ISADOR LADOFF, OF CLEVELAND, OHIO, ASSIGNOR OF THIRTY ONE-HUNDREDTHS TO  
PHILIP C. PECK, OF NEW YORK, N. Y.

## ARC-LIGHT ELECTRODE.

1,025,407.

Specification of Letters Patent.

Patented May 7, 1912.

Application filed June 1, 1907. Serial No. 376,868.

To all whom it may concern:

Be it known that I, ISADOR LADOFF, a citizen of the United States, and a resident of the city of Cleveland, county of Cuyahoga, 5 and State of Ohio, have invented certain new and useful Improvements in Arc-Light Electrodes, of which the following is a specification, reference being had to the accompanying drawings, in which—

10 Figure 1 is a perspective view of one of my pencils and Fig. 2, a central longitudinal section of Fig. 1.

My present improvements relate particularly to arc lights for metallic, or essentially 15 metallic pencils, that is to say pencils composed of metal, or preponderantly of metal, and a principal object of my invention is to adapt such pencils to produce, readily, in the alternating current, well defined, long, quiet, and exceptionally luminous arcs, though my said pencils are also well adapted to be used in a continuous current.

The opinion has, I believe, been hitherto 25 universal that the alternating current cannot, with practical and industrial success, be maintained between non-carbon pencils. I have discovered that the aforesaid objects of my present invention can be attained 30 and metallic pencils successfully used in the alternating current by bringing salts into the presence of the molten metal at the upper surface of such pencils in such current, which I secure by imparting to such 35 pencils a cylindrical form, *i. e.*, a central longitudinal bore and filling the latter with salts of alkaline, or electropositive metals, such as on the one hand sodium or potassium salts, preferably potassium fluorid, or 40 on the other hand salts of cæsium, rubidium, calcium.

The pencils may be made of the metal desired in any convenient way; they are then drilled or otherwise treated, to produce 45 the bore into which is packed the coring of salts, as aforesaid. Those skilled in the art will readily understand how, in the case of different metals, to determine the best proportions of core and pencil relatively to each other; also how best in each

case to produce the hollow pencils and insert the coring. For example: I have produced what may be termed an essentially metallic pencil as follows: I mixed together with oxid of titanium enough pulverized 55 magnetite to insure presence in the pencil produced as hereinafter described of at least 60 parts metallic iron and oxid of titanium, 40 parts. To the mixture I added as a binder, a small proportion of water, sufficient to impart to the powder adhesion and plasticity. I then squirted and molded the plastic mass into the forms required for the pencils, these being cylinders of about eight (8") inches long and one-half (½") 60 inch diameter. After drying in the open air for several hours, the pencils were further dried in an oven at a temperature of about 200 degrees centigrade for some forty-eight hours. They were then packed in carbon, 65 and subjected for about eight (8) hours to a temperature of from 1200 degrees to 1500 degrees centigrade, the magnetite being thus substantially reduced to metallic iron, and the finished pencils composed preponderantly 70 of iron, the pencils having a diameter of about  $\frac{1}{2}$ " and a bore of 0.185 inch in diameter. This bore was packed full of potassium fluorid. In arcing, the described pencils were used as cathode and anode. An 75 alternating current being turned on, 4 amperes and 80 to 90 volts drop across the arc, the resulting arc was readily maintained indefinitely. It was of superior luminosity, well defined, long and quiet. Of course the 80 said metallic pencils may be prepared in any other convenient manner, the essential point being to provide them with a core of salts as stated.

I am aware that carbon pencils, mineralized carbon pencils, and the like have been previously cored, also, that salts have been incorporated into such pencils, and therefore do not broadly claim coring, or the introduction of salts into pencils generally. 90

What I claim as new and desire to secure by Letters Patent is the following:—

1. A metallic arc light pencil comprising a bore containing potassium fluorid.
2. An essentially metallic arc light pencil 100

composed preponderantly of iron and comprising a bore containing potassium fluorid.

3. A metallic arc light pencil comprising a core composed of potassium fluorid.

4. An arc-light pencil composed preponderantly of metal in elemental state and comprising a central longitudinal bore containing a salt of an alkaline metal.

5. An arc-light pencil composed preponderantly of iron in elemental state and comprising a central longitudinal bore containing a salt of an alkaline metal. 10

ISADOR LADOFF.

Witnesses:

F. W. SINRAM,  
R. P. MEQUILLET.